

# United States Patent Office

2,694,017

Patented Nov. 9, 1954

1

2,694,017

## PROCESS OF CHEMICAL NICKEL PLATING OF ALUMINUM AND ITS ALLOYS AND BATHS THEREFOR

Raymond R. Reschan, East Chicago, and Abraham Krieg, Gary, Ind., assignors to General American Transportation Corporation, Chicago, Ill., a corporation of New York

No Drawing. Application September 16, 1952,  
Serial No. 309,939

10 Claims. (Cl. 117—50)

The present invention relates to improved processes of chemical nickel plating of aluminum and its alloys employing baths of the nickel cation-hypophosphite anion type, and to improved baths employed in such processes.

The chemical nickel plating of any catalytic material, including aluminum and its alloys, employing an aqueous acid bath of the nickel cation-hypophosphite anion type is based upon the catalytic reduction of nickel cations to metallic nickel and the corresponding oxidation of hypophosphite anions to phosphate anions with the evolution of hydrogen gas at the catalytic surface. The reactions take place when the body of catalytic material is immersed in the bath, and the exterior surface of the body of catalytic material is coated with nickel. The chemical nickel plating process is autocatalytic since both the original surface of the body being plated and the nickel metal that is deposited on the surface thereof are catalytic; and the reduction of the nickel cations to metallic nickel in the bath proceeds until all of the nickel cations have been reduced to metallic nickel, in the presence of an excess of hypophosphite anions, or until all of the hypophosphite anions have been oxidized to phosphate anions, in the presence of an excess of nickel cations. Actually the reactions are slowed down rather rapidly as time proceeds because the anions, as contrasted with the cations, of the nickel salt that is dissolved in the bath combine with the hydrogen cations to form an acid, which, in turn, lowers the pH of the bath, tending to dissolve the nickel deposit. Also the reducing power of the hypophosphite anions is decreased as the pH value of the bath decreases. Moreover, there is a tendency for the bath, as the pH value thereof is decreased, to become unstable with the formation of a "black precipitate" that comprises a random chemical non-catalytic reduction of the nickel cations; which formation of the "black precipitate" is also favored by a high absolute concentration of hypophosphite anions in the bath. Of course, this formation of "black precipitate" comprises a decomposition of the bath, and is further objectionable in that it causes the nickel deposit to be coarse and rough.

For the dual purposes of increasing the stability of the bath (preventing the formation of the "black precipitate" mentioned) and of increasing the normal plating rate of the bath, various baths of the present type have been suggested employing different additives that serve either as buffers or as exaltants. For example, in U. S. Patent No. 2,532,283, granted on December 5, 1950, to Abner Brenner and Grace E. Riddell, there are shown two chemical nickel plating baths of the aqueous acid nickel cation-hypophosphite anion type that respectively contain as buffer additives sodium acetate and sodium citrate; and in the copending application of Gregoire Gutzeit and Ernest J. Ramirez, Serial No. 204,424, filed January 4, 1951, now Patent No. 2,658,842, granted November 10, 1953, there are disclosed a number of chemical nickel plating baths of the aqueous acid nickel cation-hypophosphite anion type that contain as exaltant additives various salts of simple short chain saturated aliphatic dicarboxylic acids, including sodium succinate.

While the above-mentioned stabilized baths of the nickel cation-hypophosphite anion type are well-suited to the chemical nickel plating of such catalytic materials as copper, chromium, cobalt, iron, nickel and palladium, they are not ideally suited to the chemical nickel plating

2

ing of aluminum and its alloys, since aluminum and its alloys are attacked by the bath due to its low pH (acid corrosion); and since the reactions involved proceed too violently bringing about an early formation in the baths of the "black precipitate" and the resulting coarse, rough and dark nickel deposits on the body being plated and formed essentially of aluminum or the alloys thereof.

The present invention involves the discovery that in the chemical nickel plating of aluminum and its alloys, a bath of the nickel cation-hypophosphite anion type may be readily stabilized by employing as an additive a small amount of a soluble nitrate, such as sodium nitrate, potassium nitrate, nickel nitrate, etc. It is postulated that the nitrate anions "inhibit" the catalytic surface of the aluminum or aluminum alloy body resulting in a decrease of the effective reducing power of the hypophosphite anions. In any case, a bath of the character noted containing the nitrate additive mentioned results in the chemical nickel plating of aluminum and its alloys at a satisfactory rate and without the formation of the "black precipitate" in the bath, whereby the nickel deposit is smooth and bright. Also, it has been discovered that the plating rate of such a stabilized bath of the character described may be greatly increased, without inducing instability therein, by employing as an additional additive, a small amount of a soluble fluoride, such as sodium fluoride, potassium fluoride, etc. The combination in the nickel cation-hypophosphite anion bath of the nitrate and the fluoride additives brings about in the chemical nickel plating of aluminum and its alloys a great stability of the bath and a high nickel plating rate, rendering such baths ideally suited to commercial chemical nickel plating of bodies formed essentially of aluminum or aluminum alloys.

It is, therefore, the primary object of the present invention to provide an improved chemical process of plating with nickel, aluminum and its alloys, in which the reactions involved are carried out more efficiently and perfectly than heretofore, thereby rendering the process more desirable from a commercial standpoint.

Another object of the invention is to provide an improved process of the character described that employs a bath of the nickel cation-hypophosphite type containing as an additive nitrate anions.

Another object of the invention is to provide an improved process of the character described that employs a bath of the nickel cation-hypophosphite anion type containing as additives both nitrate anions and fluoride anions.

A further object of the invention is to provide improved aqueous acid baths of the character described that are particularly well-suited to the chemical nickel plating of aluminum and its alloys.

These and other objects and advantages of the present invention will be understood from the foregoing and following description.

In accordance with the process of the present invention, the article formed essentially of aluminum or an aluminum alloy that is to be nickel plated is first properly prepared by mechanically cleaning, degreasing and light pickling. This preliminary preparation of the article is very important since it is essential to good adhesion of the nickel deposit. The pretreatment of the article may be fundamentally in accordance with standard practice in electroplating processes; and the following pretreatment is recommended as it has been found to be highly satisfactory.

First, the article is suitably cleaned of any scale or foreign matter, and then subjected to a standard vapor degreasing step. Next, the article is pickled for about 30 seconds in an aqueous hydrochloric acid solution, about 1:1 at approximately 60° C., or somewhat more concentrated at a lower temperature. The article is then rinsed with water (preferably hot), and then immersed for about 30 seconds in an aqueous solution of approximately 3 parts concentrated nitric acid (38% HNO<sub>3</sub>) and 1 part concentrated aqueous hydrofluoric acid. Finally, the article is again rinsed with water (preferably hot), and immediately immersed in a hot plating bath of the nickel cation-hypophosphite anion type of the character noted and of a composition more fully described hereinafter.

## 3

the bath being maintained at a temperature  $98^{\circ} \pm 1^{\circ}$  C. under standard conditions of pressure.

Almost immediately hydrogen bubbles are formed on the catalytic surface of the article and escape in a steady stream from the bath, while the surface of the article is slowly coated with metallic nickel. Actually the coating or deposit on the surface of the article constitutes an alloy of nickel and phosphorus containing about 3% to 8% phosphorus, by weight, but has the appearance of metallic nickel and is considered to be a metallic nickel deposit for the purpose of the disclosure of the present invention. In general, best chemical nickel plating results are obtained when the ratio (V/A) between the volume of the bath (cm.<sup>3</sup>) and the surface area of the article being plated (cm.<sup>2</sup>) is below 10.

With respect to the composition of the bath, it essentially comprises an aqueous acid solution containing nickel cations, hypophosphite anions and nitrate anions, and may be formed by dissolving in a suitable acid water solution, a soluble nickel salt, a soluble hypophosphite, and a soluble nitrate. For example, the nickel cations may be derived from nickel chloride (a commercial grade), the hypophosphite anions may be derived from sodium, potassium, calcium, magnesium, barium, etc., hypophosphites, or various combinations thereof; and the nitrate anions may be derived from sodium, potassium, nickel, etc., nitrates, or various combinations thereof. In passing, it is noted that certain alkaline cations that may be thus introduced into the bath appear to retard in the process the rate of nickel deposition with respect to other cations; for example, barium cations appear to retard the rate of nickel deposition with respect to sodium and potassium cations. Specifically, a suitable bath may be formed in an exceedingly simple manner by dissolving in a hydrochloric acid water solution commercial nickel chloride, sodium hypophosphite and sodium nitrate. The desired pH of the bath may be established by the introduction thereto of additional hydrochloric acid and may be appropriately adjusted by the addition thereto of a weak alkali, preferably sodium bicarbonate. Also, it will be understood that the nitrate anions and some of the hydrogen cations may be derived by introducing nitric acid, instead of sodium nitrate, into the bath, although ordinarily, it is easier to employ sodium nitrate for the primary purpose noted.

Also, as explained more fully hereinafter, the nickel plating rate upon aluminum and its alloys of a bath of the character above described may be materially increased by providing therein fluoride anions; which may be readily accomplished by adding a soluble fluoride to the bath in the preparation thereof. Specifically, the fluoride anions may be derived from sodium, potassium, etc., fluorides, or various combinations thereof. Also, it will be understood that the fluoride anions and some of the hydrogen cations may be derived by introducing hydrofluoric acid, instead of sodium fluoride, into the bath; although ordinarily it is easier to employ sodium fluoride for the primary purpose noted.

The terms "cations," "anions" and "ions" as employed herein include the total quantity of the corresponding elements that are present in the bath; i. e., both undissociated and dissociated material. In other words, 100% dissociation is assumed when the terms noted are used in connection with molar ratios and concentrations in the various baths.

For the purpose of demonstrating the stabilizing effect of nitrate anions upon chemical nickel plating baths of the aqueous acid nickel cation-hypophosphite anion type, a series of comparative nickel plating tests were conducted employing baths of the character of those set forth in the previously mentioned Brenner and Riddell patent.

Specifically, a first series of chemical nickel plating baths were prepared that contained the recommended ingredients, parts by weight:

Nickel chloride (NiCl<sub>2</sub>.6H<sub>2</sub>O) ----- parts--  
Sodium hypophosphite (NaH<sub>2</sub>PO<sub>2</sub>.H<sub>2</sub>O) ----- parts--  
Sodium citrate (2(Na<sub>3</sub>C<sub>6</sub>H<sub>5</sub>O<sub>7</sub>).11H<sub>2</sub>O) ----- parts--  
pH ----- 5.30-5.35  
Temperature ----- °C-- 96

A second series of chemical nickel plating baths were prepared that contained the recommended ingredients, parts by weight:

Nickel chloride (NiCl<sub>2</sub>.6H<sub>2</sub>O) ----- parts--

## 4

Sodium hypophosphite (NaH<sub>2</sub>PO<sub>2</sub>.H<sub>2</sub>O) ----- parts-- 1  
Sodium acetate (NaC<sub>2</sub>H<sub>3</sub>O<sub>2</sub>.3H<sub>2</sub>O) ----- do ----- 1.5  
pH ----- 5.30-5.35  
Temperature ----- °C-- 96

Also, there were prepared a third series of chemical nickel plating baths (identical to the first series set forth above), but also containing 0.35 mole/liter of nitrate anions derived from sodium nitrate; and a fourth series 10 of chemical nickel plating baths (identical to the second series set forth above), but also containing 0.35 mole/liter of nitrate ions derived from sodium nitrate.

Employing these four series of chemical nickel plating 15 baths, plating tests were conducted employing samples formed of aluminum and aluminum alloys that were properly pretreated, in the manner previously described. The series of samples comprised the aluminum and aluminum alloys as follows: 2-S, 25-S, 52-S and 61-S.

In each case, employing the first and second series of 20 chemical nickel plating baths above set forth, a violent reaction took place at the catalytic surface of the sample, and the bath was decomposed within a few minutes (2 to 3 minutes). In other words, each of the chemical nickel 25 plating baths in the first and second series above described was decomposed after a few minutes by the random reduction of the nickel cations to metallic nickel with the formation of "black precipitate," whereby the bath was rapidly exhausted of its nickel cation content, with no or 30 very little and spotty nickel plating. In each case, employing the third and fourth series of chemical nickel plating baths above set forth, a gentle reaction took place at the catalytic surface of the sample; the bath was not decomposed by the formation of "black precipitate"; and the nickel plating produced upon the sample was good. 35 However, the plating rate was very slow, less than 0.0001" per hour.

These sets of comparative tests clearly demonstrate that the addition of the soluble nitrate is effective in the preventing of decomposition of the bath by random reduction 40 of the nickel cations therein and the consequent formation of "black precipitate" when the bath is employed in the nickel plating of aluminum and its alloys. It is postulated that the addition of the soluble nitrate probably results in "inhibition" of the catalytic surface of the 45 sample, formed essentially of aluminum or of aluminum alloys, resulting in an effective decrease of the reducing activity of the hypophosphite anions.

Still other comparative tests of the character set forth above were conducted for the purpose of determining the proper content of the nitrate anions, and it was discovered that a large excess of nitrate anions unduly slows down the reaction, whereas an insufficient amount of nitrate anions is not adequate to prevent the random reduction of the nickel cations with the consequent formation of the "black precipitate" (metallic nickel sponge). Specifically, it was discovered in a bath of the character specified that the slow-down of the reactions 50 was unduly objectionable when the content of the nitrate anions was in excess of about 0.50 mole/liter, and that the formation of the "black precipitate" was not inhibited when the content of the nitrate anions was below about 0.15 mole/liter.

The stability of a fast chemical nickel plating bath of the character of that disclosed in the previously-mentioned Gutzeit and Ramirez application is also enhanced in a similar manner by the addition of nitrate anions thereto; which increased stability of the chemical nickel 55 plating bath results in a slow-down of the reactions as indicated by the following test:

70 A 2-S aluminum sample with a surface area of 20 cm.<sup>2</sup> was immersed in 50 cc. of an aqueous acid plating solution (C/A-2.5), heated to and maintained at  $98^{\circ}$  C., that contained the following ingredients:

|                                                | Mole/liter |
|------------------------------------------------|------------|
| Nickel cations derived from nickel chloride    | 0.09       |
| Hypophosphite anions derived from sodium hy-   |            |
| popphosphite                                   | 0.225      |
| Succinate anions derived from sodium succinate | 0.06       |
| Nitrate anions derived from sodium nitrate     | 0.35       |

The initial pH of this bath was 4.6; and the weight gain of the sample in 10 minutes was 0.0775 gm., corresponding to a nickel plating rate in gm/cm.<sup>2</sup>/min. of  $3.87 \times 10^{-4}$ .

In order to increase the nickel plating rate still further,

the above-mentioned chemical nickel plating bath was modified by the addition of fluoride anions, in the manner disclosed in the copending application of Gregorie Gutzeit Serial No. 283,825, filed April 23, 1952. Specifically, the above-mentioned bath was modified by the addition thereto of 0.02 mole/liter of fluoride anions derived from sodium fluoride; and a test identical to that described above was repeated. In this test, the weight gain of the 2-S aluminum sample was 0.0815 gm. in 10 mins., corresponding to the rate of nickel plating in gm./cm.<sup>2</sup>/min. of  $4.06 \times 10^{-4}$ .

A further series of nickel plating tests were conducted with the view of determining the best perimeters of the chemical nickel plating bath with regard to the content of nitrate anions and fluoride anions, with reference to the different aluminum alloys, and it was discovered that in each case best chemical nickel plating was obtained upon the various aluminum and aluminum alloy samples when the temperature of the bath was maintained at approximately 98° C., and the pH of the bath was adjusted within the relatively narrow range 4.5 to 4.7 employing hydrochloric or lactic acid, and that in general the composition of the bath should be:

|                           | Mole/liter   |
|---------------------------|--------------|
| Nickel cations-----       | 0.09         |
| Hypophosphite anions----- | 0.225        |
| Succinate anions-----     | 0.06         |
| Nitrate anions-----       | 0.18 to 0.35 |
| Fluoride anions-----      | 0.01 to 0.04 |

Further, it was discovered that the optimum concentration of nitrate anions in the general range 0.15 to 0.50 mole/liter was a function of the aluminum or the aluminum alloy being nickel plated; and the specific compositions with reference to content of nitrate anions of the bath corresponding to aluminum and aluminum alloys are recommended as follows:

|                          | Mole/liter<br>of NO <sub>3</sub> <sup>-</sup> |
|--------------------------|-----------------------------------------------|
| 2-S aluminum-----        | 0.18 to 0.22                                  |
| 52-S aluminum alloy----- | 0.28                                          |
| 24-S aluminum alloy----- | 0.35                                          |
| 61-S aluminum alloy----- | 0.35                                          |

Further, it was discovered that the concentration of fluoride anions in the baths should range from about 0.01 to 0.04 mole/liter; that amounts of fluoride anions in the bath in excess of about 0.04 mole/liter are practically without additional effect upon the nickel plating rate, although they are not objectionable; and that amounts of fluoride anions less than 0.01 mole/liter are without any practical effect upon the nickel plating rate.

In carrying out the foregoing approximately determined perimeters, a number of samples of 2-S aluminum having an area of 20 cm.<sup>2</sup> were pretreated, as previously described, and plated at 98° C. in an aqueous acid bath of the character mentioned containing the following ingredients:

|                           | Mole/liter |
|---------------------------|------------|
| Nickel cations-----       | 0.09       |
| Hypophosphite anions----- | 0.225      |
| Succinate anions-----     | 0.06       |
| Nitrate anions-----       | 0.35       |
| Fluoride anions-----      | 0.02       |

These baths were prepared employing commercial nickel chloride, sodium hypophosphite, sodium succinate, sodium nitrate and sodium fluoride. In four tests employing the 2-S aluminum samples mentioned, the following results were obtained:

|                                                              | 4.60   | 4.60   | 4.60   | 4.60   |
|--------------------------------------------------------------|--------|--------|--------|--------|
| Initial pH-----                                              | 4.60   |        |        |        |
| Final pH-----                                                | 3.13   | 3.12   | 3.00   | 2.04   |
| Plating time (mins.)-----                                    | 10     | 10     | 120    | 120    |
| Weight gains (gm.)-----                                      | 0.0906 | 0.0881 | 0.1800 | 0.1761 |
| Plating rate, gm./cm. <sup>2</sup> /min. $\times 10^4$ ----- | 4.33   | 4.40   |        |        |

Also from these tests, it was determined that both high nickel plating rates and great bath stability were obtained when the initial pH of these baths is in the approximate range 4.0 to 5.5, the optimum pH range being from about 4.5 to about 4.7.

In conclusion, it is pointed out that the utilization of these chemical nickel plating baths essentially comprising nickel cations, hypophosphite anions, succinate anions, nitrate anions and fluoride anions, above described,

brings about the plating of bright, smooth nickel deposits upon articles, formed of aluminum and the various alloys of aluminum, at a very satisfactory plating rate; and the nickel deposits are intimately and tenaciously bonded to the articles provided the articles are properly pretreated, as previously described. However, in the absence of proper pretreatment of the articles, poor adhesion of the nickel coatings thereon results.

In view of the foregoing, it is apparent that there has been provided an improved process of chemically plating articles formed essentially of aluminum and aluminum alloys, with nickel, and an improved bath of the nickel cations-hypophosphite anion type that is expressly useful in the plating of aluminum and its alloys, wherein the bath is of a stable composition and the nickel plating rate thereof is greatly increased with respect to prior processes of this character, by virtue of the incorporation in the bath of the nitrate anions or the combination of the nitrate anions and the fluoride anions.

While there has been described what is at present considered to be the preferred embodiment of the invention, it will be understood that various modifications may be made therein, and it is intended to cover in the appended claims all such modifications as fall within the true spirit and scope of the invention.

- What is claimed is:
1. The process of chemically plating with nickel a body essentially formed of a material selected from the group consisting of aluminum and its alloys, which comprises contacting said body with a bath consisting essentially of an aqueous solution of a nickel salt and a hypophosphite and a nitrate, wherein the absolute concentration of nitrate anions in said bath expressed in mole/liter is between 0.15 and 0.50.
  2. The process set forth in claim 1, wherein the initial pH of said bath is in the approximate range 4.0 to 5.5.
  3. The process of chemically plating with nickel a body essentially formed of a material selected from the group consisting of aluminum and its alloys, which comprises contacting said body with a bath consisting essentially of an aqueous solution of a nickel salt and a hypophosphite and a nitrate and also containing a fluoride, wherein the absolute concentration of nitrate anions in said bath expressed in mole/liter is between 0.15 and 0.50, and wherein the absolute concentration of fluoride anions in said bath expressed in mole/liter is between 0.01 and 0.04.
  4. The process set forth in claim 3, wherein the initial pH of said bath is in the approximate range 4.0 to 5.5.
  5. The process of chemically plating with nickel a body essentially formed of a material selected from the group consisting of aluminum and its alloys, which comprises contacting said body with a bath consisting essentially of an aqueous solution of a nickel salt and a hypophosphite and a nitrate and also containing a fluoride and a succinate, wherein the absolute concentration of nitrate anions in said bath expressed in mole/liter is between 0.15 and 0.50, and wherein the absolute concentration of fluoride anions in said bath expressed in mole/liter is between 0.01 and 0.04.
  6. The process set forth in claim 5, wherein the ratio between nickel cations and hypophosphite anions in said bath expressed in molar concentrations is between 0.25 and 0.60, wherein the absolute concentration of hypophosphite anions in said bath expressed in mole/liter is between 0.15 and 0.30, wherein the absolute concentration of succinate anions in said bath expressed in mole/liter is at least 0.05, and wherein the initial pH of said bath is in the approximate range 4.0 to 5.5.
  7. A bath for the chemical nickel plating of aluminum and its alloys consisting essentially of an aqueous solution of a nickel salt and a hypophosphite and a nitrate, wherein the absolute concentration of nitrate anions in said bath expressed in mole/liter is between 0.15 and 0.50.
  8. A bath for the chemical nickel plating of aluminum and its alloys consisting essentially of an aqueous solution of a nickel salt and a hypophosphite and a nitrate and also containing a fluoride, wherein the absolute concentration of nitrate anions in said bath expressed in mole/liter is between 0.15 and 0.50, and wherein the absolute concentration of fluoride anions in said bath expressed in mole/liter is between 0.01 and 0.04.
  9. A bath for the chemical nickel plating of aluminum and its alloys consisting essentially of an aqueous solution of a nickel salt and a hypophosphite and a nitrate

and also containing a fluoride and a succinate, wherein the absolute concentration of nitrate anions in said bath expressed in mole/liter is between 0.15 and 0.50, and wherein the absolute concentration of fluoride anions in said bath expressed in mole/liter is between 0.01 and 0.04.

10. The process of chemically plating with nickel a body essentially formed of a material selected from the group consisting of aluminum and its alloys, which comprises thoroughly degreasing and cleaning said body, then pickling said body in hydrochloric acid, rinsing said body in hot water, then immersing said body in an aqueous solution of nitric acid and hydrofluoric acid, again rinsing said body in hot water, and finally immersing said body in a bath consisting essentially of an 15

aqueous solution of a nickel salt and a hypophosphite and a nitrate, wherein the absolute concentration of nitrate anions in said bath expressed in mole/liter is between 0.15 and 0.50.

5  
References Cited in the file of this patent

## UNITED STATES PATENTS

| Number    | Name      | Date           |
|-----------|-----------|----------------|
| 1,045,718 | Marino    | Nov. 26, 1912  |
| 1,614,684 | Pacz      | Jan. 18, 1927  |
| 2,217,921 | Saukaitic | Oct. 15, 1940  |
| 2,296,884 | Thompson  | Sept. 29, 1942 |
| 2,532,283 | Brenner   | Dec. 5, 1950   |
| 2,580,773 | Heiman    | Jan. 1, 1952   |